

# UNITED STATES PATENT OFFICE.

LOUIS FENN VOGT, OF WASHINGTON, PENNSYLVANIA, ASSIGNOR TO STANDARD CHEMICAL COMPANY, OF WASHINGTON, PENNSYLVANIA.

## ALLOY.

1,304,224.

Specification of Letters Patent.

Patented May 20, 1919.

No Drawing.

Application filed March 11, 1918. Serial No. 221,718.

*To all whom it may concern:*

Be it known that I, Louis F. Vogt, a citizen of the United States, and a resident of Washington, in the county of Washington, 5 ton and State of Pennsylvania, have invented certain new and useful Improvements in Alloys; and I do hereby declare the following to be a full, clear, and exact description of the invention, such as will enable 10 others skilled in the art to which it appertains to make and use the same.

This invention relates to an improvement in alloys, one object of the invention being to so improve the physical properties of 15 aluminum and aluminum alloys as to enhance the strength and toughness thereof and render the same eminently useful for various purposes for which aluminum and aluminum alloys now in use are not satisfactory and efficient.

With this and other objects in view, the invention consists in an alloy as hereinafter set forth and pointed out in the claims.

The invention further consists of an alloy 25 comprising aluminum having alloyed therewith from .05 per cent. to two per cent. of uranium.

In producing my improved aluminum product, I may first make an alloy of 30 aluminum and uranium having a high content of uranium, and then employing this product as a vehicle for introducing a small amount of uranium into aluminum so that it will become thoroughly distributed throughout the aluminum and become alloyed therewith. In making the aluminum-uranium alloy having a high content of uranium and which may be considered to be an alloy in concentrated form, I may employ a process

40 wherein uranium oxid may be mixed with aluminum and subjected to reduction at a proper temperature. An example of such a process may consist in first melting aluminum by any convenient means, such as 45 in a crucible in a gas furnace and protected by a suitable slag; then a mixture of uranium oxid and aluminum shot may be

introduced into the molten aluminum bath, when a reduction of uranium oxid, will take place, with a liberation of considerable heat 50 due to the reduction of uranium oxid by aluminum. For example, for twenty-four pounds of aluminum melted in a bath, there could be used approximately sixteen pounds of aluminum shot mixed with ten 55 pounds of uranium oxid analyzing about eighty to eighty-five per cent.  $U_3O_8$ . This will result in an aluminum-uranium alloy containing approximately fifteen per cent. uranium. The concentrated alloy or product may be incorporated into the mass of 60 aluminum by introducing it into a bath of aluminum so that the uranium will become distributed throughout and become alloyed with the entire mass of aluminum in the 65 proportion of from .05 per cent. to two per cent. uranium content.

I have found that the addition of uranium to aluminum and aluminum alloys imparts to the same properties which cannot otherwise be obtained (particularly it adds materially to the strength and toughness of the metal and alloys), and it affects the micro structure favorably.

Uranium is known to be a good de-oxidizer 75 and it is believed to have considerable affinity for nitrogen. Aluminum is believed to contain considerable quantities of nitrogen, depending somewhat on the method of melting and the temperature to which it is 80 heated and uranium is believed to have influence in deoxidizing and denitrogenizing aluminum.

Having fully described my invention, what I claim as new and desire to secure by 85 Letters-Patent, is:—

1. An alloy having high qualities of strength and toughness comprising aluminum and uranium, the main body of the alloy consisting of aluminum and the uranium being in a relatively small proportion.

2. An alloy having high quality of strength and toughness, comprising aluminum and uranium, the aluminum com-

posing the major portion of the alloy and the uranium content being less than approximately two per cent.

3. An alloy having high quality of strength and toughness, comprising aluminum and uranium, the uranium being in the proportion of from approximately .05 to approximately 2 per cent.

In testimony whereof, I have signed this specification in the presence of two subscr- 10  
ing witnesses.

**LOUIS FENN VOGT.**

Witnesses:

**C. E. HOLDER,  
ALEX. McMORRAN.**